

1

2,873,182

## MOTOR FUEL

Milton Kosmin, Dayton, Ohio, assignor to Monsanto Chemical Company, St. Louis, Mo., a corporation of Delaware

No Drawing. Application December 29, 1953  
Serial No. 401,093

20 Claims. (Cl. 52--5)

The present invention relates to a special fuel suitable for use in jet and reciprocating engines, particularly as employed in various types of aircraft.

An object of the invention is to provide a supplementary emulsion fuel for jet and reciprocating engines to provide the increased power necessary for aircraft take-offs and emergency combat operations. It is also an object of the present invention to provide an emulsion fuel which will provide water to cool the interior of combustion zones of engines operating under high temperature conditions. It is a further object to provide emulsions which may be prepared with water, such as may be found in various localities with varying amounts and types of impurities.

The use of water injection in the operation of jet and reciprocating engines for emergency combat operations and increased power required in take-offs provides increased thrust due to both the increased volume and velocity of the gases discharged from the engine.

It has now been found that the use of water in emulsion form is especially advantageous for the present purpose. It has also been found that a specific combination of emulsifiers makes it possible to provide an emergency fuel from (1) a hydrocarbon fuel boiling in the motor fuel boiling range ordinarily employed for jet and reciprocating engines, together with (2) water such as may be naturally available containing various impurities occurring in such natural water.

The use of the above-described emulsion of a hydrocarbon fuel boiling in the motor fuel boiling range together with water for direct injection in jet or reciprocating engines results in a reduction of the temperature of the fuel-air charge and also by direct cooling of the combustion zone. In case of the reciprocating engines such direct cooling occurs in the cylinder, making it possible to obtain a greater power output from the engine. It is also found that reduction of carbon deposition occurs in the use of water as above described.

The present emulsions may also be employed in order to further after-burning in the operation of jet engines. Thus, the engine may be operated in accordance with the method wherein fuel is separately introduced into the gas stream after the primary combustion zone in order to complete the combustion and to create a large amount of exit gas from the jet engine. In this way, the thrust obtained may also be increased, for example, in take-offs and under combat conditions in which additional power is required. The present emulsion has the advantage that such supplementary fuel may be provided directly from the conventional hydrocarbon fuel and water so that only the emulsifying agent need be provided as a minor constituent together with commonly available water to provide the supplementary emulsion fuel.

The method for employing the present emulsion fuel in order to suppress carbon formation and to cool the interior combustion zones of jet and reciprocating engines during operation thereof comprises the introduction of

2

oxygen-containing gas and hydrocarbon fuel into a combustion zone and adding thereto an aqueous emulsion comprising from 5% to 60% by weight of hydrocarbons boiling in the motor fuel boiling range, 22% to 94.8% of

5 water and 0.1% to 6% of an emulsifying agent selected from the group consisting of (a) alkaline salts of sulfated condensation product of tridecanol or other Oxo alcohols as described herein with from 1 to 10 moles of ethylene oxide; (b) alkaline salts of dihexyl sulfophthalate; and (c) condensation products of tridecanol or other Oxo alcohols as described herein; and mixtures of two or three of the above groups of (a), (b) and (c).

10 The hydrocarbon fuel employed as one of the constituents of the emulsions defined in the present invention may be a paraffinic or naphthenic type boiling in the motor fuel boiling range, and generally characterized by an extremely low pour point. A typical hydrocarbon fuel of this type for jet engines is a low vapor pressure liquid made from a mixture of gasoline and cracked kerosene.

15 20 For reciprocating engines, the conventional aircraft type gasoline may be employed.

The water employed in the preparation of the present fuel combinations need not be distilled nor specifically purified but may contain naturally occurring amounts of 25 soluble salts such as carbonates, chlorides and sulfates of calcium, magnesium and sodium, such as are commonly found in hard water regions.

20 30 The emulsifying agent employed in the present emulsion fuels may be a single emulsifying component or a combination thereof. The emulsifiers employed in the present invention are (1) an alkaline salt of dihexyl sulfophthalate, such as an amine salt or butylammonium dihexyl sulfophthalate; and/or (2) an alkaline salt of the sulfated condensation product of alcohols condensed with 35 ethylene oxide. The alkaline salt of the sulfated condensation product is based upon the ethylene oxide addition product with a highly branched monohydric primary alcohol having the molecular configuration of an alcohol produced by the Oxo process from an olefin such as triisobutylene and tetrapropylene with from 1 to 10, preferably 1 to 5 moles of ethylene oxide per mole of alcohol. A preferred embodiment in the present invention is the use of a mixture of isomeric monohydric primary tridecyl alcohols, said alcohols being derived from the catalyzed 40 45 Oxo reaction of carbon monoxide and hydrogen with a material of a class consisting of polyisobutylenes and polypropylenes. The third component is (3) an ethylene oxide condensation product of tridecanol with 1-10 moles of ethylene oxide.

50 55 When polymer olefins such as polyisobutylene or polypropylene are reacted according to the Oxo reaction with carbon monoxide and hydrogen in the presence of the catalyst containing cobalt carbonyl, thorium and magnesium oxides or allied catalytic materials, a mixture of isomeric alcohols having a wide boiling range is obtained. The alcohols may be manufactured by the process described in the United States Bureau of Mines Report of Investigation No. 4270, dated June 1948. In view of the presence of a number of isomers of triisobutylene or tetrapropylene, for example, in the polymer olefins which are treated according to the Oxo reaction and furthermore since there is considerable isomerization, polymerization and depolymerization of the olefins due to the catalytic action, the resulting alcoholic product contains a large 60 65 number of different alcohols, some of which are polyhydric alcohols. By reason of the large number of compounds present in the Oxo reaction product it has so far been impossible to ascertain the exact composition of this product.

70 75 The formation of the present condensation products is carried out by passing ethylene oxide either as a gas or as a liquid into the Oxo alcohol, such as tridecyl al-

cohol in the presence of an alkaline catalyst such as caustic soda or potash. Using from 0.25% to 1.5% by weight of the catalyst based on the alcohol is satisfactory. The condensates are then sulfated by conventional methods, after which the sulfated product is neutralized to form the alkaline salt, such as the sodium, potassium, ammonium or an alkyl amine salt. The amine salt may be prepared by the use of mono-, di- or trimethylamines or the corresponding ethyl or ethanolamines.

In preparing the mixture of the said emulsifying agents of the two types described above, it has been found that the proportion thereof may vary from 0.3:1 to 4:1 parts by weight of the said phthalate to the said condensation product, a preferred ratio being equal proportions by weight. In the preparation of the emulsion fuels of the present invention it has been found that emulsions may desirably be prepared in the proportion of 88 parts by weight of water with 12 parts of the hydrocarbon and emulsifier. However, the present emulsions may contain from 22% to 94.7% water; 5% to 60% of the hydrocarbon and 0.1% to 6% of the emulsifier.

The examples below illustrate some of the specific embodiments of the present invention.

#### Example 1

An emulsion was prepared by mixing the following:

|                                                                                                                | Percent |
|----------------------------------------------------------------------------------------------------------------|---------|
| Hydrocarbon fuel                                                                                               | 11.4    |
| Butylamine salt of dihexyl sulfophthalate                                                                      | 0.3     |
| Sodium salt of sulfated tridecanol-1 mole ethylene oxide condensation product (alcohol derived by Oxo process) | 0.15    |
| Tridecanol-1 mole ethylene oxide condensation product (alcohol derived by Oxo process)                         | 0.15    |
| Water (300 p. p. m. hardness)                                                                                  | 88.0    |

The above combination was tested to determine the stability of the emulsion as formulated above and also with each of the surface-active agents present alone with the oil and water. The emulsion stability data for the above examples are set forth below:

| Emulsifying Agent                                                                                                                                    | Percent Liquid Separated From Emulsion |
|------------------------------------------------------------------------------------------------------------------------------------------------------|----------------------------------------|
| Combination of agents below                                                                                                                          | 1                                      |
| Butylamine salt of dihexyl-4-sulfophthalate                                                                                                          | 7                                      |
| Sodium salt of sulfated tridecanol-ethylene oxide condensation product (5:1 molar ratio) with tridecanol-5 moles ethylene oxide condensation product | 10                                     |

The measure of emulsion stability as employed in the present test is the amount of liquid separated after 20 hours of standing at 30° C.

It is obvious from the above results that the combination of the surface-active agents in the emulsion fuel results in a product having greater stability than can be obtained from a single surface-active agent employed alone. When the ethylene oxide condensation product with tridecanol (or other Oxo alcohols) is employed with the sodium salt of a sulfated condensation product of this type it is preferred to have the former present in equal proportion to one-half as much as the sodium salt of the sulfated derivative. A typical mixture is shown in Example 1.

It has been found that the above specific emulsifying agents employed singly, as a binary system or as a ternary system results in the formation of hydrocarbon-water emulsions of the greatest utility in view of the remarkable tolerance which the said emulsions display towards water hardness and the presence of soluble salts such as are found in naturally occurring waters in various

regions. However, the present invention also contemplates the use of single emulsifiers. Examples of such emulsifiers are the alkaline salts of dihexyl sulfophthalate such as amine salts, and the alkaline salts of the sulfated condensation product of tridecanol and similar Oxo alcohols with ethylene oxide. Typical alkaline salts are the sodium, ammonium and amine salts, such as methyl, ethyl, propyl, butyl, pentyl and hexyl amine salts employed as the mono-, di-, or triamines or the corresponding alkanolamines. Another class of emulsifiers are the ethylene oxide condensation products of tridecanol and other Oxo alcohols as described above. Such latter condensation products preferably have from 1 to 10 moles of ethylene oxide per mole of the alcohol.

The emulsion-stability values of other fuels based upon various emulsifiers are set forth below:

| Emulsifiers                                                           | Conc. | Water Hardness | Percent Liquid Separated From Emulsion |         |
|-----------------------------------------------------------------------|-------|----------------|----------------------------------------|---------|
|                                                                       |       |                | 5 Min.                                 | 20 Hrs. |
| Dimethyl Amine salt of di-hexyl-4-sulfophthalate                      | 1.2   | 50             | 8                                      | -----   |
| Isopropyl Amine salt of di-hexyl-4-sulfophthalate                     | 0.6   | 50             | 0                                      | 6       |
| Butylamine salt of di-hexyl-4-sulfophthalate                          | 1.2   | 50             | 0                                      | 8       |
| Ammonium hexyl-4-sulfophthalate                                       | 1.2   | 50             | 0                                      | 2       |
| Na salt of sulfated tridecanol + 5 E. O. *                            | 1.2   | 50             | 0                                      | 1       |
| + 1 E. O. *                                                           | 1.2   | 150            | 0                                      | 7       |
| + 1 E. O. *                                                           | 1.2   | 300            | 0                                      | 7       |
| + 1 E. O. *                                                           | 1.2   | 50             | 0                                      | 8       |
| Dimethylamine salt of sulfated tridecanol + 5 E. O.                   | 1.2   | 50             | 22                                     | -----   |
| Isopropylamine salt of sulfated tridecanol + 5 E. O.                  | 1.2   | 50             | 20                                     | -----   |
| n-Butylamine salt of sulfated tridecanol + 5 E. O.                    | 1.2   | 50             | 18                                     | 10      |
| Ammonium salt of sulfated tridecanol + 5 E. O.                        | 1.2   | 50             | 0                                      | 8       |
| Butylamine salt of dihexyl-4-sulfophthalate plus tridecanol + 1 E. O. | 0.9   | 50             | 0                                      | 16      |
| Tridecanol + 5 E. O.                                                  | 0.3   | 50             | 0                                      | 16      |
| Na salt of sulfated tridecanol + 1 E. O. plus tridecanol + 1 E. O.    | 0.9   | 300            | 0                                      | 7       |
| Na salt of sulfated tridecanol + 1 E. O. plus tridecanol + 1 E. O.    | 0.3   | 300            | 0                                      | 7       |
| Na salt of sulfated tridecanol + 1 E. O.                              | 1.2   | 300            | 0                                      | 11      |

\* Contains 25% of condensation product of 1 mole ethylene oxide per mole tridecanol.

#### What is claimed is:

- An improved motor fuel which comprises from 5% to 60% of hydrocarbons boiling in the motor fuel boiling range, emulsified with 22% to 94.8% of water as the disperse phase in the presence of the combination of (a) 0.1% to 6% of an alkaline salt of dihexyl sulfophthalate together with (b) 0.1% to 6% of an alkaline salt of a sulfated condensation product of ethylene oxide with a mixture of highly-branched monohydric primary alcohols having the molar configuration of an alcohol produced by the Oxo process from an olefin of the class consisting of polyisobutylenes and polypropylenes, and (c) 0.1% to 6% of an ethylene oxide condensation product with an alcohol described in (b) which has been condensed in the presence of an alkaline catalyst selected from the group consisting of caustic soda and caustic potash.
- An improved motor fuel which comprises from 5% to 60% of hydrocarbons boiling in the motor fuel boiling range, 22% to 94.7% of water; 0.1% to 6% of butylamine salt of hexyl-4-sulfophthalate and from 0.1% to 6% of the sodium salt of the sulfated condensation product of tridecanol and ethylene oxide which has been condensed in the presence of an alkaline catalyst selected from the group consisting of caustic soda and caustic potash.
- An improved motor fuel which comprises from 5% to 60% of hydrocarbons boiling in the motor fuel boiling range, 22% to 94.7% of water, and 0.1% to 6% of a condensation product of tridecanol with from 1 to 10

moles of ethylene oxide which has been condensed in the presence of an alkaline catalyst selected from the group consisting of caustic soda and caustic potash.

4. An improved motor fuel which comprises hydrocarbons boiling in the motor fuel boiling range, emulsified with water in the presence of 0.1% to 6% of an alkaline salt of a sulfated condensation product of tridecanol with from 1 to 10 moles of ethylene oxide which has been condensed in the presence of an alkaline catalyst selected from the group consisting of caustic soda and caustic potash per mole of the said tridecanol together with 0.1% to 6% of an alkaline base salt of dihexyl sulfophthalate.

5. An improved motor fuel which comprises hydrocarbons boiling in the motor fuel boiling range, emulsified with water as the disperse phase in the presence of the combination of 0.1% to 6% of an alkaline salt of dihexyl sulfophthalate together with 0.1% to 6% of an alkaline salt of a sulfated condensation product of ethylene oxide with a mixture of highly-branched monohydric primary alcohols having the molar configuration of an alcohol produced by the Oxo process from an olefin of the class consisting of polyisobutylenes and polypropylenes which has been condensed in the presence of an alkaline catalyst selected from the group consisting of caustic soda and caustic potash.

6. An improved motor fuel which comprises from 5% to 60% of hydrocarbons boiling in the motor fuel boiling range, 22% to 94.7% of water; 0.1% to 6% of butylamine salt of hexyl-4-sulfophthalate and from 0.1% to 6% of the ethylene oxide condensation product of sulfated tridecanol which has been condensed in the presence of an alkaline catalyst selected from the group consisting of caustic soda and caustic potash.

7. An improved motor fuel which comprises from 5% to 60% of hydrocarbons boiling in the motor fuel boiling range, 22% to 94.7% of water, and 0.1% to 6% of the sodium salt of the sulfated condensation product of tridecanol with from 1 to 10 moles of ethylene oxide which has been condensed in the presence of an alkaline catalyst selected from the group consisting of caustic soda and caustic potash.

8. An improved motor fuel which comprises from 5% to 60% of hydrocarbons boiling in the motor fuel boiling range, 22% to 94.7% of water, and 0.1% to 6% of the butylamine salt of the sulfated condensation product of tridecanol with from 1 to 10 moles of ethylene oxide which has been condensed in the presence of an alkaline catalyst selected from the group consisting of caustic soda and caustic potash.

9. An improved motor fuel which comprises from 5% to 60% of hydrocarbons boiling in the motor fuel boiling range, 34% to 94.7% of water, and 0.1% to 6% of an alkaline salt of dihexyl sulfophthalate.

10. An improved motor fuel which comprises from 5% to 60% of hydrocarbons boiling in the motor fuel boiling range, 34% to 94.7% of water, and 0.1% to 6% of an amine salt of dihexyl sulfophthalate.

11. An improved motor fuel which comprises from 5% to 60% of hydrocarbons boiling in the motor fuel boiling range, 34% to 94.7% of water, and 0.1% to 6% of the butylamine salt of dihexyl sulfophthalate.

12. An improved motor fuel which comprises from 5% to 60% of hydrocarbons boiling in the motor fuel boiling range, 28% to 94.7% of water, and 0.1% to 6% of alkaline salts of the sulfated condensation product of tridecanol with from 1 to 10 moles of ethylene oxide which has been condensed in the presence of an alkaline catalyst selected from the group consisting of caustic soda and caustic potash, and alkaline salts of dihexyl sulfophthalate.

13. A method for suppressing carbon formation and cooling the interior combustion zones of jet and reciprocating engines during operation thereof, said operation including introducing oxygen-containing gas and hy-

drocarbon fuel into a combustion zone, and adding thereto an aqueous emulsion comprising from 5% to 60% of hydrocarbons boiling in the motor fuel boiling range, 28% to 94.7% of water, 0.1% to 6% of butylamine salt of dihexyl-4-sulfophthalate, and from 0.1% to 6% of the sodium salt of the ethylene oxide condensation product of sulfated tridecanol which has been condensed in the presence of an alkaline catalyst selected from the group consisting of caustic soda and caustic potash.

14. An improved motor fuel which comprises from 5% to 60% of hydrocarbons boiling in the motor fuel boiling range, 22% to 94.7% of water, and 0.10% to 6% of an alkaline salt of the sulfated condensation product of tridecanol with from 1 to 10 moles of ethylene oxide, 0.1% to 6% of an alkaline salt of dihexyl sulfophthalate, and 0.1% to 6% of a condensation product of tridecanol with from 1 to 10 moles of ethylene oxide per mole of the said tridecanol which has been condensed in the presence of an alkaline catalyst selected from the group consisting of caustic soda and caustic potash.

15. An improved motor fuel which comprises from 5% to 60% of hydrocarbons boiling in the motor fuel boiling range, 22% to 94.7% of water, and 0.1% to 6% of an alkaline salt of the sulfated condensation product of 1 to 10 moles of ethylene oxide with a mixture of highly-branched monohydric primary alcohols having the molar configuration of an alcohol produced by the Oxo process from an olefin of the class consisting of polyisobutylenes and polybutylenes, 0.1% to 6% of an alkaline salt of dihexyl sulfophthalate, and 0.1% to 6% of a condensation product of 1 to 10 moles of ethylene oxide per mole of said Oxo alcohols which has been condensed in the presence of an alkaline catalyst selected from the group consisting of caustic soda and caustic potash.

16. An improved motor fuel which comprises from 5% to 60% of hydrocarbons boiling in the motor fuel boiling range, 28% to 97% of water, and 0.10% to 6% of an alkaline salt of the sulfated condensation product of tridecanol with from 1 to 10 moles of ethylene oxide, and 0.1% to 6% of a condensation product of tridecanol with from 1 to 10 moles of ethylene oxide which has been condensed in the presence of an alkaline catalyst selected from the group consisting of caustic soda and caustic potash.

17. An improved motor fuel which comprises from 5% to 60% of hydrocarbons boiling in the motor fuel boiling range, 34% to 94.7% of water, and 0.10% to 6% of a condensation product of tridecanol with from 1 to 10 moles of ethylene oxide which has been condensed in the presence of an alkaline catalyst selected from the group consisting of caustic soda and caustic potash.

18. An improved motor fuel which comprises from 5% to 60% of hydrocarbons boiling in the motor fuel boiling range, 28% to 94.7% of water, and 0.10% to 6% of an alkaline base salt of dihexyl sulfophthalate, and 0.10% to 6% of a condensation product of tridecanol with from 1 to 10 moles of ethylene oxide which has been condensed in the presence of an alkaline catalyst selected from the group consisting of caustic soda and caustic potash.

19. An improved motor fuel which comprises from 5% to 60% of hydrocarbons boiling in the motor fuel boiling range, emulsified with 22% to 94.8% of water in the presence of (a) 0.1% to 6% of an alkaline salt of a sulfated condensation product of an Oxo alcohol with from 1 to 10 moles of ethylene oxide per mole of the said alcohol, together with (b) 0.1% to 6% of an alkaline salt of dihexyl sulfophthalate, and (c) 0.1% to 6% of a condensation product of an Oxo alcohol with from 1 to 10 moles of ethylene oxide, the said condensation being conducted with an alkaline catalyst selected from the group consisting of caustic soda and caustic potash.

20. An improved motor fuel which comprises from 5% to 60% of hydrocarbons boiling in the motor fuel boiling range, emulsified with 22% to 94.8% of water

in the presence of (a) 0.1% to 6% of an alkaline salt of a sulfated condensation product of tridecanol with from 1 to 10 moles of ethylene oxide per mole of the said tridecanol, together with (b) 0.1% to 6% of an alkaline salt of dihexyl sulfophthalate, and (c) 0.1% to 6% of a condensation product of tridecanol with from 1 to 10 moles of ethylene oxide, the said condensation product being obtained in the presence of an alkaline catalyst selected from the group consisting of caustic soda and caustic potash.

5  
10

## References Cited in the file of this patent

## UNITED STATES PATENTS

|           |              |               |
|-----------|--------------|---------------|
| 1,935,264 | Felix et al. | Nov. 14, 1933 |
| 2,111,100 | Kokatnur     | Mar. 15, 1938 |
| 2,603,557 | Roush        | July 15, 1952 |

## FOREIGN PATENTS

|         |               |               |
|---------|---------------|---------------|
| 213,628 | Great Britain | Mar. 31, 1924 |
| 879,689 | France        | Nov. 30, 1942 |